

Aug. 23, 1938.

F. R. HENSEL ET AL

2,127,596

ALLOY

Filed June 15, 1937



*Fig. 1*

COLD WORK AFTER  
AGEING.



*Fig. 2*

ELECTRICAL CONDUCTIVITY  
& HARDNESS VS. AGEING  
TIME

QUENCHED FROM 950°C  
AGED AT 450°C

HARDNESS - ▲  
CONDUCTIVITY - ○



*Fig. 3*

HARDNESS VS. AGEING &  
COLD WORK AFTER AGEING

QUENCHED FROM 900°C  
AGED AT 450°C

INVENTORS  
Franz R. Hensel  
BY Earl J. Larsen  
B. F. Robins  
ATTORNEY

## UNITED STATES PATENT OFFICE

2,127,596

## ALLOY

Franz R. Hensel and Earl I. Larsen, Indianapolis,  
Ind., assignors to P. R. Mallory & Co., Inc.,  
Indianapolis, Ind., a corporation of Delaware

Application June 15, 1937, Serial No. 148,284

5 Claims. (Cl. 148—32)

This invention relates to alloys, and more particularly to copper alloys of improved characteristics. The object of the invention is to produce an improved copper base alloy.

Another object is to produce a copper magnesium alloy of comparatively low magnesium content, which can be hardened by means of the addition of a small percentage of zirconium to a higher degree than has heretofore been possible.

Another object is to produce a copper alloy which has an excellent combination of hardness, electrical conductivity and resistance to annealing.

Specific objects are the provision of improved copper-zirconium-magnesium alloys especially suitable for fabrication into welding electrodes, high strength sand castings for use with cylinder heads, pistons and other parts of internal combustion engines, commutator segments, trolley wires, collector rings, switch plates, bolts, nuts and in general for all uses where high strength and/or high conductivity are required at elevated temperatures.

Other objects of the invention will be apparent from the following description taken in connection with the appended claims.

The present invention comprises a combination of elements, methods of manufacture and the product thereof brought out and exemplified in the disclosure hereinafter set forth, the scope of the invention being indicated in the appended claims.

In the drawing:

Fig. 1 is a graph illustrating the effect of cold working of the alloy referred to in Fig. 2 after aging.

Fig. 2 is a graph showing a curve illustrating the improvement during age hardening in the hardness and electrical conductivity of an alloy composed of

|           |         |                          |
|-----------|---------|--------------------------|
| Magnesium | Percent | 0.45                     |
| Zirconium | Percent | 0.86                     |
| Balance   | Percent | substantially all copper |

Figure 3 is a graph showing a curve illustrating the improvement in hardness during aging of an alloy composed of

|           |         |                          |
|-----------|---------|--------------------------|
| Magnesium | Percent | 1.33                     |
| Zirconium | Percent | 1.13                     |
| Balance   | Percent | substantially all copper |

and also showing the effect of cold working of the alloy after aging.

According to our invention, we provide an

alloy of copper, magnesium and zirconium in the following permissible range of proportions:

|           | Percent              |
|-----------|----------------------|
| Magnesium | 0.05 to 3            |
| Zirconium | 0.1 to 10            |
| Balance   | substantially copper |

The preferred range of proportions are as follows:

|           | Percent              |
|-----------|----------------------|
| Magnesium | 0.1 to 1.5           |
| Zirconium | 0.1 to 2             |
| Balance   | substantially copper |

In some instances it may be desirable for certain uses to effect an improvement in the alloy by adding small percentages of additional ingredients, such as silver, zinc, tin, cadmium, calcium, lithium, silicon, titanium, beryllium and aluminum.

In carrying out the present invention a copper magnesium alloy may first be made according to the conventional alloy making procedure of the prior art and then the zirconium may be added.

It is also possible, however, to produce a copper-zirconium alloy first by melting down the copper and adding the zirconium in the form of a hardener alloy which may contain anywhere from 5-50% zirconium. This hardener alloy can be either a pressed product or a pressed and sintered product or a melted product. The magnesium is preferably added also in the form of a hardener alloy. Magnesium, in addition to its function as an alloying ingredient, will also act as a very strong deoxidizer and therefore with this new combination of copper magnesium zirconium it is possible to produce very sound castings.

After the alloy has been prepared according to such alloying methods as described above, the heat treatment may be carried out as follows:

The alloy in the form of a billet or a sand casting or any other form, is raised in temperature above 700 degrees C., and preferably to a temperature within the range of 800-1000 degrees C. The alloy is then quenched from this high temperature and subsequently aged at a temperature below 700 degrees C., and preferably in the range between 400-600 degrees C. It is possible to cold work the alloy after the complete heat treatment.

In many instances, we have found it advisable to cold work the alloy after quenching, then subsequently age it, with or without further cold working after aging. We have found it possible to eliminate quenching operations and cold work the material after hot working and subsequently

age in the range specified above. This latter treatment will usually not give as good results as the first treatment. Alloys produced according to this treatment will show a Rockwell B hardness of over 80 and an electrical conductivity of over 60%, international annealed copper standard. Alloys of the nature described will retain these properties when heated to temperatures up to 500 degrees C.

10 Copper-magnesium alloys containing considerable percentages of zirconium will not soften but will retain the hardness almost indefinitely. This is of great importance whenever the alloy is being used at elevated temperatures. Usually 15 copper base alloys, particularly when cold worked, lose their hardness at elevated temperatures and it is necessary to apply additional cold work to raise the hardness to the original value. At the same time, the elastic and tensile properties are 20 decreased considerably. Therefore, copper alloys have been very limited as structural parts in machinery which is run at elevated temperatures. The new alloy described in the present disclosure provides a material, which on account of its 25 strength at elevated temperature and its good thermal conductivity, will provide an excellent material for such structural parts. Furthermore, alloys of the type described have a high resistance to oxidation and to corrosion.

30 While, for instance, it is necessary to add as much as 10% aluminum to obtain a certain oxidation resistance of a copper base alloy, the combined presence of 2% magnesium and zirconium will provide the same resistance.

35 Alloys prepared as indicated above are well suited for the manufacture of any type of castings, such as sand castings, chill castings or permanent mold castings. The alloys are further well suited for such manufacturing processes as 40 extruding, forging, rolling and drawing. On account of the combination of high hardness, high electrical and high thermal conductivity,

the material can be used for electrical parts of any description.

Another important use for these high strength copper base alloys is in the fabrication of parts of internal combustion engines, such as automobile engines where high heat conductivity is 5 needed.

While the present invention as to its objects and advantages has been described herein as carried out in specific embodiments thereof, it is not 10 desired to be limited thereby, but it is intended to cover the invention broadly, within the spirit and the scope of the appended claims.

What is claimed is:

1. An alloy containing about 0.05 to 3.0% magnesium, 0.1 to 10% zirconium, and the remainder copper. 15

2. An age hardened alloy containing about 0.05 to 3% magnesium, 0.1 to 10% zirconium, and the remainder substantially all copper, characterized 20 by a combination of high hardness and high electrical conductivity and further characterized by the ability to maintain its hardness and high electrical conductivity at temperatures in the order of 500° C. 25

3. An electrical current carrying member composed of about 0.05 to 3% magnesium, 0.1 to 10% zirconium, and the remainder copper. 30

4. A heat conducting member composed of about 0.05 to 3% magnesium, 0.1 to 10% zirconium, and the remainder copper. 35

5. A welding electrode composed of about 0.05 to 3.0% magnesium, 0.1 to 10% zirconium, and the remainder substantially all copper, characterized by a combination of high hardness and high electrical conductivity, and further characterized by the ability to maintain its hardness and high conductivity at temperatures in the order of 500° C. 40

FRANZ R. HENSEL. 40  
EARL I. LARSEN.